

Nov. 24, 1936.

F. R. RAPIDS

2,061,591

ELECTROLYTIC DEVICE

Filed March 21, 1935



Inventor  
Felix R. Rapids.

By Charles Phillips Atty.

Patented Nov. 24, 1936

2,061,591

# UNITED STATES PATENT OFFICE

2,061,591

## ELECTROLYTIC DEVICE

Felix R. Rapids, Chicago, Ill.

Application March 21, 1935, Serial No. 12,209

3 Claims. (Cl. 204—5)

This invention relates to an electrolytic device and more particularly to a device for effecting the electrodeposition of metals or for use in the stripping of a metal from a metal coated article.

5 More particularly, the invention relates to a device in the nature of a brush for use with a relatively viscous solution of an electrolyte in the application of a metal coating by brushing the solution of the electrolyte over the surface of the article to be coated while at the same time passing an electric current through the solution of the electrolyte to the work and thereby effecting a deposition of a metal.

It is an important object of this invention to 15 provide a device for the electrolytic deposition or removal of metals that does not require the use of a stationary bath of the electrolyte but which permits the carrying out of the operation upon either small or large articles regardless of whether they are portable or not.

20 It is a further important object of this invention to provide a device in the nature of a brush for the effecting of the electrodeposition of metals in much the same manner as one would apply a paint or the like.

25 It is a further important object of this invention to provide a portable device that may be employed in electrodepositing metals upon permanently positioned metal structures that would otherwise require the dismantling of the structures if the usual plating baths were to be employed.

30 Other and further important objects of this invention will be apparent from the disclosures in the specification and the accompanying drawing.

35 This invention (in a preferred form) is illustrated in the drawing and hereinafter more fully described.

40 On the drawing:  
Figure 1 is a longitudinal sectional view of a device embodying the principles of my invention, with parts in elevation and with the electrical circuit shown diagrammatically.

45 Figure 2 is a plan view of the device.  
Figure 3 is an enlarged sectional view taken substantially on the line III—III of Fig. 1.

As shown on the drawing:  
The reference numeral 10 indicates generally 50 a brushing device embodying the principles of my invention and comprises a handle 11, a bristle brush 12 and a metal ferrule 13 encasing the upper ends of the bristles and secured to the handle 11 by means of rivets 14, or similar fastening means. The handle 11 is of suitable electrical

insulating material, such as wood, molded plastic, a rubber compound, or the like. The brush proper 12 may be composed of animal bristles, fiber bristles or strands of metal wire, or any suitable medium capable of a brushing, wiping or 5 scouring action may be employed.

The rivets 14 also serve to secure to the ferrule 13 a spring contact member 15 having at its free end a finger button 16 providing a contact point 17 adapted to be spring pressed against a 10 second contact point 18 affixed to the handle 11. Said handle 11 is suitably provided with a longitudinally extending bore 19 through which extends a wire 20 that is connected to the contact point 18. The function of the manually operable switch S, provided by the member 15 and contact points 17 and 18, is to permit the electrolyte to be brushed on first with the current off and then, by closing the switch, to carry out the 15 plating operation. The switch, however, is not 20 absolutely essential.

A battery 21 provides a source of electrical current for operating the device. Either one or more dry cells may be conveniently used, or for heavier work, it may be desirable to use wet cells 25 or other source of current. Instead of being separate from the brushing device 10, the battery 21 may comprise one or more dry cells that are contained within or attached to the handle 11.

A work block 22, which serves to support and 30 form contact with a work piece 23 is connected to the negative side of the battery 21 by means of a wire 24 and a contact post 25. The work block 22 may be entirely eliminated and the wire 24 connected directly to the work piece 23, as by 35 means of a clamp, by soldering or other suitable means.

In using the brushing device of my invention, the brush 12 is first dipped into a solution of an electrolyte, a portion of which is picked up by 40 the brush and adheres thereto as a film or mass 26. Said film of electrolyte 26 extends from the metal ferrule 13 to the surface of the work 23 that is to be coated or from which a metal coating is to be stripped. When the switch S is closed, the 45 electrical circuit from the battery 21 is thus complete through the wire 20, the contact points 18 and 17, the spring contact member 15, ferrule 13 and electrolyte 26 to the work 23. The other side of the circuit is completed through the work 50 block 22, the binding post 25 and wire 24.

In the plating operation, the metal of the ferrule 13 forms the anode and may serve to supply metal to the electrolyte composition to replace that which is electrodeposited onto the work. 55

- Practically any metal may be used, such as zinc, copper, cadmium, nickel, tin, iron, lead, chromium, and others. It is not necessary, however, that the metal of the ferrule be the same as that to be electrodeposited since the active electrolyte can always be replenished by repeated dippings of the brush applicator into the electrolyte composition. Consequently, the anode may be lead, iron, tin, or any other suitable metal, regardless of the particular metal to be electrodeposited. The solution of the electrolyte 26 is composed of an aqueous, alkaline or acid solution of a compound capable of furnishing ions of the metal to be plated out.
- 15 In order to insure a complete circuit through the electrolyte solution, it is preferable to employ a solution of a relatively viscous nature as compared with the usual electrolyte solutions of plating baths. Such a solution may be prepared by 20 dissolving any suitable metallic compound, salt, or the like, in a water or acid solution and adjusting the solution to the desired viscosity, using as a thickening agent, such materials as starch, gums, sugars, gelatin, petroleum jelly, or the like. By incorporating these or similar thickening agents, in proportions of between 2.5 and 40% by weight, say, the viscosity of the electrolyte may be built up to any desired extent, ranging from a thin syrupy consistency to a semi-solid, or jell.
- 25 The viscosity of the electrolyte solution should be such that it does not run too much on the work and make the operation a sloppy one, but will adhere to vertical surfaces, to projections and the like. The lower limit of viscosity appears to 30 be about 100 secs. (Saybolt Universal at 62° F.). This is at least twice the viscosity of the usual plating baths.
- 35 As a specific example of a suitable electrolyte solution, the following composition is given, in which the percentages are expressed as percentages by weight:

|                                        | Percent |
|----------------------------------------|---------|
| Nickel chloride (NiCl <sub>2</sub> )   | 25      |
| Ammonium chloride (NH <sub>4</sub> Cl) | 10      |
| 45 Cornstarch                          | 20      |
| Water                                  | 45      |

The above composition of the electrolyte solution is merely by way of exemplification, since obviously any suitable ionizable metal compound or salt can be used, depending upon the particular metal to be electrodeposited. As is well understood by those skilled in the art, electro-deposition of the metal from the electrolyte occurs upon the closing of the circuit and this metal is constantly replenished by metal from the ferrule 13.

60 The bristles of the brush 12 serve not only to spread the electrolyte over the surface of the work 23 but also have a brushing or scouring action that aids in the removal of foreign particles, oxides, and the like, from the surface of the work. It is, however, preferable to clean the work before applying the electrolyte solution and this may be accomplished in any of the usual manners, as by scouring, pickling, abrasion, or the like.

65 After the work has been cleaned, the electrolyte solution is brushed onto the work, with the switch S open, to a uniform thickness. This aids in obtaining a uniform coating, since it gives the electrolyte an opportunity to thoroughly cover and wet the surface of the work. The current may, however, be kept on from the start, if de-

sired. One advantage of the use of a flexible brush is that the electrolyte solution may be readily coated over irregular surfaces and carried into deep indentations, depressions and similar points of the surface contour.

5 After the electrolyte solution has been brushed on, the circuit is closed and the brushing continued to accomplish the plating operation. The thickness of the coating of metal plated out in this manner will obviously be governed by the 10 time of application, the current density, the concentration of the metal compound in the electrolyte solution and other conditions known to those skilled in the plating art. In order to get a good, even and uniform plate, the brush strokes should 15 be regular and even and should cover the entire surface that it is desired to coat. After the plating operation is complete, the layer of electrolyte solution may be wiped or washed off and the work piece washed.

20 Where the device is to be used to strip a metal coating of a plated article, the current is reversed. In this case, the nature of the electrolyte is more or less immaterial, since the solution of the electrolyte merely serves to complete the circuit to transfer the metal stripped from the work to the ferrule. The electrolyte solution should, of course, have sufficient body to adhere to the brushing agency and complete the circuit.

25 The use of a thickening agent in the electrolyte 30 solution seems to have the added function of absorbing or adsorbing the hydrogen that may be liberated during the plating operation, since I have observed that there is practically no gassing and no trouble from polarization, using my 35 process. The main function, however, of the thickening agent is to give the electrolyte solution sufficient body that it will adhere to the brushing element and form a continuous electrical circuit between the metal anode or cathode and the work 40 to be plated.

30 I am aware that many changes may be made and numerous details of construction may be varied through a wide range without departing from the principles of this invention, and I, therefore, do not purpose limiting the patent granted hereon otherwise than necessitated by the prior art.

45 I claim as my invention:

1. A device for use in the electrodeposition of 50 metals, comprising a brush having a handle and bristles attached thereto, a metal ferrule encasing the attached end of said bristles, an electrical conductor in electrical contact with said ferrule and a manually operable make-and-break mechanism carried by said handle for connecting said conductor to a source of current.

55 2. A device for use in the electrodeposition of metals, comprising a brush having a handle and bristles attached thereto, a metal ferrule encasing 60 the attached end of said bristles, a spring contact member secured to said ferrule, a contact carried by said handle for cooperation with said member and a wire extending along said handle from said contact for connection to a source of current.

65 3. A brush for use in the electrodeposition of metals, comprising a handle, bristles extending from one end thereof, a metal ferrule encasing 70 said end and extending into contact with and overlying said bristles and an electrical conductor connected to said ferrule.

FELIX R. RAPIDS.